

# UNITED STATES PATENT OFFICE.

PIERCE D. SCHENCK, OF DAYTON, OHIO, ASSIGNOR TO THE DURIRON COMPANY, INC.,  
A CORPORATION OF NEW YORK.

## HEAT-RESISTING IRON.

1,398,917.

Specification of Letters Patent. Patented Nov. 29, 1921.

No Drawing.

Application filed April 12, 1920. Serial No. 373,326.

To all whom it may concern:

Be it known that I, PIERCE D. SCHENCK, a citizen of the United States, and a resident of Dayton, in the county of Montgomery and State of Ohio, have made a new and useful Invention in Heat-Resisting Iron, of which the following is a specification.

The invention relates to an alloy which is largely iron, and which will resist a high degree of heat, so that the composition may be loosely termed a heat resisting iron. The invention is designed to take the place of the relatively expensive compositions now on the market and containing relatively high proportions of the rare metals. The primary ingredients of the composition are iron, nickel and chromium, the latter being used in relatively small quantities, so that the composition may be used for many purposes where other compounds having approximately the same heat resisting qualities cannot be used because of the prohibitive cost. A further object of the invention is the production of a composition or alloy of the character above specified, which can be machined without difficulty, being like cast iron in such respect; which is not brittle, being in fact somewhat malleable; which is acid resisting to a high degree, and which is relatively tough.

In its best form the composition contains about 85 parts of iron, 5 to 15 parts of nickel and 1 to 3 parts of chromium. As a specific example, a very satisfactory composition comprises 10 parts of nickel, 2 parts of chromium, and the balance iron. In making the compound an electric or open hearth furnace is preferably employed, the chromium being added in the form of ferro chrome and melted with the iron. The bath is then skimmed and the nickel added.

The iron employed is low in silicon, preferably less than 1%, as any amount over 1% tends to injure the acid and heat resisting qualities of the composition. The iron is also preferably low in carbon, preferably 1 to 1½% or less. The composition thus produced is relatively cheap and will stand 2200 degrees F. without oxidization and 2600 degrees F. without melting. It is tough and somewhat malleable, can be easily cast and

machined, and has high acid resisting qualities. The field of use is therefore very wide. It will be understood that the proportions specified may be varied somewhat without departing from the invention, and also that certain other ingredients of more or less neutral character may be added without greatly affecting the quality of the product. For instance, cast iron normally contains a small percentage of manganese as an impurity and some other impurities in minute quantities, which do not affect the composition appreciably. The invention comprehends the use, incidental or otherwise, of such ingredients. In fact I have found that even additional manganese may be added without injuring the composition to any extent, although I prefer to omit such element because it involves no advantage and means additional expense. There are many other elements which can similarly replace a portion of the iron and are more or less neutral in their effect upon the iron and acid resisting qualities of the composition. The term "iron" therefore is not limited to pure 100% iron but comprehends iron with such expected impurities as do not unfit it for its intended use and iron containing small percentages of other metals which are more or less neutral in their effect upon the composition resulting.

I have found that the proportions of nickel and chromium as heretofore specified give a product which best suits the requirements for which the iron is intended, viz. one which has great heat and acid resisting qualities, combined with toughness and of just the right degree of hardness to permit machining without brittleness. If more nickel is added, the composition is softened and made of too great price for general use. If decreased below the amount specified, the composition becomes too hard and brittle and lacks the desired degree of toughness. Similarly, if the chromium is increased, the composition is hardened so that it is difficult to machine, without increasing the heat and acid resisting qualities, and the cost increased. A lowering of the amount of chromium reduces the heat and acid resisting qualities below the desired point.

What I claim is:

1. A heat resisting iron composition comprising approximately 10 per cent. nickel, 2 per cent. chromium and the rest substantially all iron.

2. A heat resisting iron composition comprising approximately 10 per cent. nickel,

2 per cent. chromium and the rest substantially all iron with any silicon content in the iron less than 1 per cent.

In testimony whereof, I have hereunto subscribed my name this 30th day of March, 1920.

PIERCE D. SCHENCK.